# EUROPEAN PATENT SPECIFICATION

(11) **EP 0 356 066 B1**
(45) Date of publication and mention of the grant of the patent: **08.04.1992**
(21) Application number: 89308088.7
(22) Date of filing: 09.08.1989
(51) Int. Cl.: E01C 7/26, E01C 7/35, E01C 11/16, E01C 11/12, E01D 19/06

(54) **Improved material for bridge joints and for use in, and method of, repairing or surfacing roads and the like**
Materialien für Brückenfugen und zur Verwendung beim Reparieren oder Verkleiden von Strassen und dergleichen und Verfahren
Matériaux pour joints de ponts, l'utilisation dans et procédé pour la préparation ou le revêtement des chaussées et similaires

(30) Priority: 26.08.1988 GB 8820329; 28.12.1988 GB 8830290
(43) Date of publication of application: 28.02.1990
(73) Proprietor: FIBRESCREED LIMITED, Uckfield East Sussex TN22 1QL (GB)
(72) Inventor: McIntosh, James, East Sussex (GB); Goodenough, Ronald James, Nr Haywards Heath East Sussex (GB)
(74) Representative: Williams, Trevor John

(56) References cited:
- CH-A- 539 003
- GB-A- 2 048 904
- US-A- 4 265 563
- US-A- 4 440 816

## Description

This invention relates to an improved material and process using this material to repair or surface roads, parking areas, aircraft pavements and other load bearing areas. For example, the method may be applied to aircraft pavements, roads, paths, motorways and footpaths. The material may also be used to provide a flexible bridge joint filler or expansion joint in a multistorey car park or other structure.

The present invention, in one aspect, is particularly concerned with providing repairs using a material which has some degree of resilience and which has a tensile strength and is thus especially useful where the surface to be repaired is jointed or cracked or spalled. This is particularly useful where one is endeavouring to repair concrete surfaces or surfaces with a concrete underlay in that the concrete expands and contracts greatly with changes of temperature and if one uses a conventional road surfacing material this is brittle and the movement of the concrete tends to provide reflective cracks from the joints or cracks in the concrete to the surface of the black top, Macadam or other conventional surfacing material. Thus, frequently with old concrete surfaces which have been laid in concrete with expansion joints between adjacent concrete areas, not only do the joints themselves cause difficulty but after a period of use the edges of the joints frequently will crack and one can end up with a substantial degree of cracking or enlargements of the joints and spalling of the concrete, that is the provision of localised crack holes and hollows in the concrete, which, if filled with conventional materials will permit the ready transference of cracks to the applied surfacing material after a relatively small period of use.

The present invention is concerned with the provision of a material which uses rubber to give the necessary resilience, which may have aggregate included to provide improved load bearing resistance and which also includes material to provide a tensile strength.

EP-A-0 202 966 discloses a material in accordance with the prior art portion of claim 1. While it is known to use rubber chips obtained from old rubber tyres for binding such bituminous material in the manufacture of road repairing material, in general it has been ensured that any wire reinforcing material is removed so that the material salvaged from the tyres is simply the rubber chips. Also, it has been proposed in GB-A-2 048 904 to provide wire reinforcements in a bituminous surfacing which is a substantially rigid mixture of aggregate and length wire bound with bituminous material. Surprisingly, the present invention, as specified in claim 1 has found it advantageous to use the wire reinforcement in a material which is inherently resilient without loss of resilience and with a considerable improvement in the strength and wear-resisting properties. The simple operation of chopping up the wire-reinforced rubber tyres, as well as forming the chips, unravels the wire reinforcement and cuts that down to lengths, substantially longer than the chip dimension, which are ideal for the required strengthening purposes, without unduly reducing the flexibility of the material.

Generally, when referring herein to rubber chips, we are concerned with rubber in the form of pieces having a maximum dimension greater than 2 mm, preferably in the range of 3 to 7 mm, conveniently about 5 mm. However, where the material is used to a substantial depth, for example to fill a groove at a bridge or other joint, the chips may have a greater maximum dimension, for example 15 mm or even 20 mm. Generally, also, the metal fibre or wire is very fine and is chopped to have a length greater than the rubber chip dimensions.

A further aspect of the invention provides a method of repairing or surfacing roads, parking areas and other load bearing areas in which the hot material of the invention is applied to the area. In most cases aggregate is mixed with the bituminous binder, which itself may be rubberised bitumen including 5 to 25% rubber, and chopped glass or other fibres may in some circumstances also be mixed therewith although not normally required.

Where one is using the material of the present invention to repair localised areas of joints or cracking or spalling, the aggregate may be included up to as much as 25 mm in maximum dimension although preferably it will be from 3 to 5 mm in maximum dimension to ease application, especially where the depth of application in some areas is quite small. Once the sites of movement, for example expansion joints and cracks, have been covered with the material, possibly strengthened with aggregate, and reinforced with the metal fibre or wire a covering overlay may be applied to render the area fit for use. Typically, this overlay may be of glass fibre strengthened bitumen with a surface dressing as disclosed in GB-A-2 081 603. Alternatively, a conventional black top or Macadam surface may be applied to a thickness 30 mm, more usually in excess of 50 mm, frequently as much as 100 or 200 mm. Other alternative surface overlays or dressings which may be used include veneer surfacings of 3 mm upwards in thickness and a mixture of the bituminoos binder material, rubber chips and metal fibre or wire.

Where one is using the material of the invention with the inclusion of aggregate to cover a surface area, the aggregate should have a maximum dimension of 5 mm, preferably approximately 3 mm, and generally no larger than the dimensions of the rubber chips in the material. Such a layer would be particularly suitable for spreading on more lightly loaded paths and the like, where the underlying surface may be crazed or lightly cracked or which has had more badly damaged areas already repaired and filled otherwise, for example with the material of the invention which contains a greater proportion of rubber in the bitumen and possibly larger sized aggregate.

The material of the invention may be mixed on site or may be supplied ready mixed for subsequent melting down and laying.

We will describe, by way of example, the use of material of the present invention for repairing joints and cracked or spalled surfaces or providing thin patches to badly worn localised areas. In doing this, the material may typically comprise approximately 50% of rubberised bitumen binder material. The rubberised bitumen binder will have added to it 5 to 50% by weight rubber chips and metal fibre or wire which has been formed by the coarse chopping of vehicle tyres. By chopping metal reinforced tyres an appropriate proportion of metal reinforcement wire or fibre is provided for the mix. During this chopping of the tyres the metal reinforcing strands in the tyre become untwisted and unravelled and are chopped but, because of their flexibility and fineness, the individual lengths of wire are left with a length several times the dimension of the rubber chips. For use in patching purposes one would expect at least 10%, preferably 15%, rubber in the rubberised bitumen. The aggregate could have a maximum dimension of preferably 3 to 5 mm although, depending upon the circumstances, a greater maximum dimension could be used, for example even as much as 20 to 25 mm. Where additional fibre, preferably glass, is added to the mixture it would not normally be more than 5% and in most cases 0.5 to 1.5%, say 1%, is adequate, in those unusual situations where tensile strength additional to that provided by the metal is required. The hot mixture is applied to the cracks or other surface areas requiring substantial repair and when set the additional covering surface is applied as required. Thus, as indicated previously, this additional surface may, for example, be a glass fibre reinforced bitumen provided with a dressing or a conventional black top Macadam surface. The resilience of the rubber chips in the bitumen with the tensile strength provided by the chopped metal fibre or wire prevents reflective cracks passing from the underlaying repaired surface to the top surface of the overlay and the substantial aggregate content of the material enables it to be load bearing and resistant to subsidence when passed over by heavy vehicles. A relatively thin layer of this material may be applied over localised areas for patching purposes as a membrane subsequently to be covered by an overlay.

In a situation where the material of the present invention is being used to form a bridge joint or an expansion joint in a large structure, for example a multistorey garage, in general no aggregate will be used in the mixture which will comprise a major proportion of the rubber chips bound, preferably, with a resilient bitumen material such as a polymer modified bitumen. When repairing such a joint, a groove will be provided spanning the joint and this groove will be filled with the material of the invention level to the surface on either side of the groove and a further surface layer for supporting the traffic will then be provided over the joint and over the structure on either side of the joint. In such a location where the depth of the groove may be quite substantial, the rubber chips may well have a maximum dimension as big as 15 mm, perhaps as much as 20 mm. The material can either be applied hot and rolled in situ or where the groove can be cut accurately, the material may be provided as preformed strips, insertable in the cut grooves. While, preferably, no aggregate is included in the material as used for repairing bridge or expansion joints, in some cases where the reduced flexibility can be tolerated, a proportion of aggregate may be used in the filling mixture.

Generally, above, we have been referring to the use of a material comprising the rubber chips and metal fibres mixed therein for localised patching purposes, normally prior to subsequent covering with a traffic bearing overlay surface. However, the present invention can also be used to provide an overall layer or membrane over an entire base area with that membrane layer including the rubber chips and the fine metal fibre or wire reinforcement. This can be achieved simply by spreading a layer of rubberised bitumen or rubberised polymer modified bitumen over the area, the rubberised bitumen preferably, although not necessarily, including a fine aggregate or sand filler. The rubber chips and metal reinforcement can either be mixed in that rubberised bitumenous layer prior to application of the material or may be distributed over the material after it has been laid and then rolled and compressed so as to become embedded in that material in the same manner that in a more conventional road surfacing aggregate would be spread over and compressed into an underlying binding layer. One disadvantage of using rubberised bitumen as the binder material, although adding to the resilience and quantity of rubber in the layer, is that it cannot be applied easily by spraying. Thus, in an alternative method utilising the invention a less viscous, more liquid, bitumen emulsion or polymer modified bitumen emulsion may be sprayed over the surface prior to having the rubber chips and metal reinforcement distributed thereover for rolling in position. Aggregate may also be applied or included in the distributed bitumenous binder as required but normally in this situation would not have a dimension greater than that of the rubber chips and preferably would have a very much smaller dimension, more commonly being in the form of a fine grained aggregate or sand filler to the binder.

One particularly preferred method comprises distributing a layer of bitumenous binder with the addition of chopped glass fibre or other fibres and then distributing the rubber chips and metal reinforcement over that layer prior to rolling it in to cause it to be bound into a continuous rubberised layer. A further traffic bearing overlay can then be provided over the area to which the membrane has been applied.

A membrane layer as referred to above is particularly useful for applying as a thin repair layer to such surfaces as lightly loaded paths or other walk-on areas which are infrequently used by vehicles although even so the resilience of the rubber of the layer will give a resistance to cracking in conjunction with the tensile strength added by the included fibres of metal and possibly also of glass or the like.

In general, in most applications, the proportion of aggregate in the material may be from 40 to 60% although proportions outside this range may be used, depending upon the particular application and the amount of fine grained filler, if any, in the rubberised bitumen. Preferably, the proportion of aggregate in the material is approximately 50% by weight. However, in other applications no aggregate at all may be used. Thus a sandwich construction may be provided in which the sandwich "filling" comprises a membrane or layer of bitumen containing the chopped rubber pieces and metal fibre or wire. This "filling" may, or may not, contain aggregate depending upon the degree of resilience required, and provides for good non-cracking load transfer from an overlying top layer to the underlying support or base surface.

In all these applications, we have referred to glass fibres as being used when applied additionally to the metal fibres or wire. Usefully, the glass fibres may be chopped to a length of approximately 30 mm. While we have referred herein generally to the use of glass fibres, it will be appreciated that other materials may be used, for example polyamide or other metal fibres, although presently glass fibres are the preferred additional tensile-strength-imparting material when such is required.

Various advantages accrue from the use of the substantial sized pieces of rubber in the material of the present invention in conjunction with the longer lengths of fibre metal wire or fibre. Surprisingly, better wear resistance appears to be obtained than when using the simple conventional rubberised bitumen having a far smaller rubber particle size and also the incorporation of the metal wire provides very good tensile strength properties despite the relatively small proportion of metal wire present. While in some extreme cases it may be desirable to add additional longer fibres to increase tensile strength, in general it has been found that the use of the metal fibres or wires is very adequate and gives a better result than previous structure of the applicants as disclosed in GB-A-2 200 645 where smaller rubber particle sizes are used with the longer glass or other fibres providing the tensile strength. Indeed, where extreme resilience is required, the present invention can use the bitumen and rubber with the chopped wire reinforcement with very little if any aggregate addition in order to provide a resilient waterproof membrane of substantial thickness between different layers of a road or other load bearing surface.

A particular advantage of the present material is that it can very readily be made simply by chopping up old wire reinforced vehicle tyres. Thus, modern radial tyres contain a substantial amount of metal reinforcement which conventionally is very difficult to separate reliably from the rubber in order to use the rubber for other purposes, for example broken down to a small particle-sized crumb for use in conventional rubberised bitumen. The material of the present invention requires far less breaking down of the tyres in view of the relatively large rubber chip size. The inclusion of the metal of the tyre reinforcement randomly bound to or, more usually, separated from the rubber chips provides what appears to be an ideal road construction material where it is important to prevent the transmission of reflective cracks. Thus, during the chopping up of the rubber tyres the twisted tensile cables are chopped and rapidly unravelled to the very fine and flexible constituents of the cable. Due to this fineness and flexibility most of the metal is not chopped as short as the dimensions of the rubber chips such that when the rubber is formed in 2 mm dimension chips the pieces of wire will normally have a length of from 20 to 30 mm; however due to the random nature of the chopping some of the metal lengths will be shorter, similar in length to the rubber chip dimensions or even shorter.

## Claims

1. A material for use in repairing or servicing roads, parking areas, aircraft pavements and other load bearing areas, such material comprising rubber chips having a maximum dimension of at least 2 mm and a bituminous binder characterised in that mixed with the chips are lengths of metal fibre or wire longer than the maximum dimension of the chips, said rubber chips and lengths of metal fibre or wire being bound together with the binder, the binder itself being a rubberised bitumen material.

2. A material according to claim 1, wherein the bitumen of the rubberised bitumen is a polymer modified bitumen.

3. A material according to claim 2, wherein the bituminous binder is rubberised bitumen material which includes 5 to 25% rubber.

4. A material according to any preceding claim, wherein the metal fibres are approximately 20 to 30 mm long.

5. A material according to any preceding claim, which also comprises up to 5%, preferably 0.5 to 1.5%, by weight of glass or other fibres.

6. A material according to any preceding claim, wherein the rubber chips have their maximum dimensions in the range of 3 to 7 mm, preferably about 5 mm.

7. A material according to any preceding claim, wherein the bituminous binder has aggregate mixed therewith, the aggregate being no larger than 25 mm and preferably no larger than 5 mm in maximum dimension.

8. A material according to claim 7, wherein the aggregate has dimensions similar to that of the rubber chips.

9. A method of repairing or surfacing roads, parking areas, aircraft pavements and other load bearing areas in which a hot material is applied to the area, such material being as claimed in any preceding claim.

10. A method according to claim 9, wherein the material is applied to localised damaged portions only of the area.

11. A method according to claim 9, wherein the material is applied as a continuous membrane layer over the whole area.

12. A method according to claim 10 or 11, wherein the area has sequentially applied to it a covering traffic bearing overlay.

13. A method of providing a bridge joint or expansion joint wherein material as claimed in any one of claims 1 to 6 is applied to a groove spanning the joint in the bridge or other structure.

14. A method according to claim 13, wherein the material is applied hot and rolled in situ.

15. A method according to claim 13, wherein the material is applied as a preformed strip into the groove, the groove having been cut to the required size to receive the strip.

16. A method according to any one of claims 13 to 15, wherein the rubber chips have a maximum dimension of up to 20 mm.

17. A method according to any one of claims 13 to 16, wherein a traffic bearing surface layer is provided over the material of the joint and over the structure on either side thereof in which the groove is formed.

18. A method according to claim 12 or 17, wherein said surface layer is applied as a mixture of said bituminous binder material, rubber chips and metal fibre or wire.

19. A method according to claim 12 or 17, wherein the surface layer is applied by spreading a layer of bituminous binder material over the filled groove and neighbouring surface, distributing a mixture of rubber chips and metal fibre or wire over the binder material and rolling the chips and metal into the binder material to be bound thereby.

20. A method according to claim 19, wherein the bituminous binder material itself has rubber chips and metal fibre or wire mixed therein before application to the area.

21. A method according to claim 19 or 20, wherein aggregate is added by being distributed over the bituminous binder material and rolled thereinto together with the rubber chips and metal.

22. A method according to claim 12 or 17, wherein the surface layer is a black top overlay of at least 30 mm thickness.

23. A method according to claim 12 or 17, wherein the surface overlay comprises a bituminous layer strengthened with glass or other fibres and provided with a surface layer of chippings or the like.

24. A material according to any one of claims 1 to 8, or a method of any one of claims 9 to 23, wherein the rubber chips and metal fibres or wire have been obtained by chopping up wire-reinforced vehicle tyres.

## Patentansprüche

1. Material zur Verwendung bei der Ausbesserung oder Wartung von Straßen, Parkflächen, Flugzeugrollbahnen und anderen Belastung tragenden Flächen, wobei dieses Material Gummischnitzel umfaßt, die eine maximale Abmessung von zumindest 2 mm und ein bituminöses Bindemittel aufweisen, dadurch gekennzeichnet, daß Abschnitte aus Metallfaser oder Draht mit den Schnitzeln vermischt sind, die länger als die maximale Abmessung der Schnitzel sind, wobei die Gummischnitzel und die Abschnitte aus Metallfaser oder Draht über das Bindemittel miteinander verbunden sind, wobei das Bindemittel selber ein gummiertes Bitumenmaterial ist.

2. Material nach Anspruch 1, bei dem das Bitumen des gummierten Bitumen ein polymermodifiziertes Bitumen ist.

3. Material nach Anspruch 2, bei dem das bituminöse Bindemittel ein gummiertes Bitumenmaterial ist, welches 5 bis 25% Gummi umfaßt.

4. Material nach einem der vorhergehenden Ansprüche, bei dem die Metallfasern etwa 20 bis 30 mm lang sind.

5. Material nach einem der vorhergehenden Ansprüche, welches auch einen Gewichtsanteil von bis zu 5%, vorzugsweise 0,5 bis 1,5%, von Glasfasern oder anderen Fasern umfaßt.

6. Material nach einem der vorhergehenden Ansprüche, bei dem die maximalen Abmessungen der Gummischnitzel in dem Bereich von 3 bis 7 mm, vorzugsweise bei etwa 5 mm, liegen.

7. Material nach einem der vorhergehenden Ansprüche, bei dem dem bituminösen Bindemittel ein Zuschlagstoff beigemischt ist, der eine maximale Abmessung von nicht länger als 25 mm und vorzugsweise nicht länger als 5 mm aufweist.

8. Material nach Anspruch 7, bei dem der Zuschlagstoff Abmessungen aufweist, die denen der Gummischnitzel ähnlich sind.

9. Verfahren zum Ausbessern oder Herstellen von Decken von Fahrbahnen, Parkflächen, Flugzeugrollbahnen und anderen Belastung tragenden Flächen, in dem ein heißes Material auf die Fläche aufgebracht wird, wobei es sich bei dem Material um das in den vorhergehenden Ansprüchen beanspruchte handelt.

10. Verfahren nach Anspruch 9, in dem das Material nur auf eingegrenzte beschädigte Abschnitte der Fläche aufgebracht wird.

11. Verfahren nach Anspruch 9, in dem das Material in Form einer kontinuierlichen Schicht über der ganzen Fläche aufgebracht wird.

12. Verfahren nach Anspruch 10 oder 11, in dem ein den Verkehr tragender abdeckender Überzug sequentiell auf die Fläche aufgebracht ist.

13. Verfahren zur Bildung einer Brückenverbindungsstelle oder Dehnungsfuge, in dem das in einem der Anspüche 1 bis 6 beanspruchte Material auf eine Ritze aufgebracht wird, die sich über die Verbindungsstelle an der Brücke oder einer anderen Struktur erstreckt.

14. Verfahren nach Anspruch 13, in dem das Material an Ort und Stelle heiß aufgebracht und gewalzt wird.

15. Verfahren nach Anspruch 13, in dem das Material als vorgeformter Streifen in die Ritze eingebracht wird, wobei die Ritze auf die passende Größe zur Aufnahme des Streifens geschnitten worden ist.

16. Verfahren nach einem der Ansprüche 13 bis 15, in dem die Gummischnitzel eine maximale Abmessung von bis zu 20 mm aufweisen.

17. Verfahren nach einem der Ansprüche 13 bis 16, in dem eine den Verkehr tragende Deckschicht über dem Material der Verbindungsstelle und über der Struktur auf jeder Seite davon vorgesehen ist, in der die Ritze ausgebildet ist.

18. Verfahren nach Anspruch 12 oder 17, in dem die Deckschicht in Form einer Mischung aus bituminösem Bindemittelmaterial, Gummischnitzeln und Metallfaser oder Draht aufgebracht wird.

19. Verfahren nach Anspruch 12 oder 17, in dem die Deckschicht durch Ausbreiten einer Schicht von bituminösem Bindemittelmaterial über der gefüllten Ritze und der benachbarten Oberfläche, durch Verteilen einer Mischung aus Gummischnitzeln und Metallfaser oder Draht über das Bindemittelmaterial und durch Einwalzen der Gummischnitzel und des Metalls in das Bindemittelmaterial zur Verbindung damit aufgebracht wird.

20. Verfahren nach Anspruch 19, in dem dem bituminösen Bindemittelmaterial selber vor dem Auftragen auf die Fläche Gummischnitzel und Metallfaser oder Draht beigemischt werden.

21. Verfahren nach Anspruch 19 oder 20, in dem ein Zuschlagstoff hinzugefügt wird, indem er über dem bituminösen Bindemittelmaterial verteilt und dort zusammen mit den Gummischnitzeln und dem Metall hineingewalzt wird.

22. Verfahren nach Anspruch 12 oder 17, in dem die Deckschicht ein Schwarzdeckenüberzug von einer Dicke von zumindest 30 mm ist.

23. Verfahren nach Anspruch 12 oder 17, in dem der Decküberzug eine bituminöse Schicht umfaßt, die mit Glasfasern oder anderen Fasern verstärkt und mit einer Deckschicht aus Splitt oder dergleichen versehen ist.

24. Material nach einem der Ansprüche 1 bis 6 oder Verfahren nach einem der Ansprüche 9 bis 23, in dem die Gummischnitzel und Metallfasern oder Draht durch Zerhacken von drahtverstärkten Fahrzeugreifen erhalten worden sind.

## Revendications

1. Matériau destiné à être utilisé pour la réparation ou l'entretien de routes, aires de stationnement, voies de roulement d'avions et autre zones de support de charge, ce matériau comprenant des copeaux de caoutchouc dont la dimension maximale est d'au moins de 2 mm, et un liant bitumineux, caractérisé en ce que des longueurs de fibres ou de fils métalliques plus longues que la dimension maximale des copeaux sont mélangées aux copeaux, lesdits copeaux de caoutchouc et lesdites longueurs de fibres ou de fils métalliques étant liés ensemble par le liant, le liant lui-même étant un matériau en bitume caoutchouté.

2. Matériau selon la revendication 1, dans lequel le bitume du bitume caoutchouté est un bitume polymère modifié.

3. Matériau selon la revendication 2, dans lequel le liant bitumineux est un matériau en bitume caoutchouté qui comprend de 2 à 25% de caoutchouc.

4. Matériau selon l'une quelconque des revendications précédentes, dans lequel les fibres métalliques ont une longueur d'approximativement 20 à 30 mm.

5. Matériau selon l'une quelconque des revendications précédentes, qui comprend également jusqu'à 5%, et de préférence de 0,5 à 1,5% en poids, de fibres de verre ou autres.

6. Matériau selon l'une quelconque des revendications précédentes, dans lequel les dimensions maximales des copeaux de caoutchouc sont situées dans la plage de 3 à 7 mm, et de préférence d'environ 5 mm.

7. Matériau selon l'une quelconque des revendications précédentes, dans lequel un agrégat est mélangé au liant bitumineux, la dimension maximale de l'agrégat étant non supérieure à 25 mm et de préférence non supérieure à 5 mm.

8. Matériau selon la revendication 7, dans lequel l'agrégat a des dimensions similaires à celle des copeaux de caoutchouc.

9. Procédé pour réparer ou entretenir des routes, des aires de stationnement, des voies de roulement d'avions et autres zones de support de charge, dans lequel un matériau chaud est appliqué sur la zone, ce matériau étant tel que revendiqué dans l'une quelconque des revendications précédentes.

10. Procédé selon la revendication 9, dans lequel le matériau est appliqué seulement dans des portions endommagées et localisées de la zone.

11. Procédé selon la revendication 9, dans lequel le matériau est appliqué sous forme d'une couche formant une membrane continue sur l'ensemble de la zone.

12. Procédé selon la revendication 10 ou 11, dans lequel une sur-couche de support de trafic est appliquée ensuite sur la zone.

13. Procédé pour réaliser un joint de pont ou un joint d'expansion, dans lequel le matériau selon l'une quelconque des revendications 1 à 6 est appliqué dans une gorge s'étendant le long d'un joint de pont ou d'une autre structure.

14. Procédé selon la revendication 13, dans lequel le matériau est appliqué à l'état chaud et roulé in situ.

15. Procédé selon la revendication 13, dans lequel le matériau est appliqué sous la forme d'une bande préformée dans la gorge, la gorge ayant été découpée à la dimension requise pour recevoir la bande.

16. Procédé selon l'une quelconque des revendications 13 à 15, dans lequel les copeaux de caoutchouc ont une dimension maximale de 20 mm.

17. Procédé selon l'une quelconque des revendications 13 à 16, dans lequel une couche de surface de support de trafic est prévue sur le matériau du joint et sur la structure, de chaque côté de celle-ci où la gorge est formée.

18. Procédé selon la revendication 12 ou 17, dans lequel ladite couche de surface est appliquée sous forme d'un mélange dudit matériau du liant bitumineux, de copeaux de caoutchouc et de fibres ou fils métalliques.

19. Procédé selon la revendication 12 ou 17, dans lequel la couche de surface est appliquée en étalant une couche du matériau formant le liant bitumineux sur la gorge remplie et la surface voisine, en répartissant un mélange de caoutchouc et de fibres ou de fils métalliques sur le matériau du liant et en incorporant par roulage les copeaux et le métal dans le matériau du liant de façon à être reliés par celui-ci.

20. Procédé selon la revendication 19, dans lequel le matériau du liant bitumineux comprend lui-même des copeaux de caoutchouc et des fibres ou fils métalliques mélangés à celui-ci, avant application sur la surface.

21. Procédé selon la revendication 19 ou 20 dans lequel un agrégat est ajouté en étant réparti sur le matériau du liant bitumineux et incorporé dans ce dernier par roulage avec les copeaux de caoutchouc et le métal.

22. Procédé selon la revendication 12 ou 17, dans lequel la couche de surface est une sur-couche noire d'une épaisseur d'au moins 30 mm.

23. Procédé selon la revendication 12 ou 17, dans lequel la surcouche de surface comprend une couche bitumineuse renforcée de fibres de verre ou autres fibres et munie d'une couche de surface en copeaux ou analogues.

24. Procédé selon l'une quelconque des revendications 1 à 8, ou procédé selon l'une quelconque des revendications 9 à 23, dans lequel les copeaux de caoutchouc et les fibres ou fils métalliques ont été obtenus par hachage de pneumatiques de véhicules renforcés de fils métalliques.
